

July 20, 1965

D. R. STERN ETAL

3,195,304

PROCESS FOR PRODUCING POWER

Original Filed July 16, 1962

2 Sheets-Sheet 1



FIG.-1

DAVID R. STERN  
ROBERT D. STEWART  
INVENTORS

BY *Wm. G. Addison*  
ATTORNEY

July 20, 1965

D. R. STERN ET AL

3,195,304

## PROCESS FOR PRODUCING POWER

Original Filed July 16, 1962

2 Sheets-Sheet 2



FIG.-2



DAVID R. STERN  
ROBERT D. STEWART

## INVENTORS

BY W. G. Addison

ATTORNEY

FIG. - 3

1

3,195,304

### PROCESS FOR PRODUCING POWER

David R. Stern, Fullerton, and Robert D. Stewart, La Habra, Calif., assignors to American Potash & Chemical Corporation, Los Angeles, Calif., a corporation of Delaware

Original application July 16, 1962, Ser. No. 209,864. Divided and this application May 1, 1964, Ser. No. 368,439

4 Claims. (Cl. 60—36)

This application is a division of application Serial No. 209,864, filed July 16, 1962, for Process and Product.

This invention relates to alkali metal alloys and to their methods of preparation. In particular, this invention relates to ternary cesium=potassium=sodium alloys and their methods of preparation.

Low melting, non-aqueous liquid heat transfer media which are liquid over a wide range of temperatures have long been sought. The present ternary alkali metal alloys provide a non-aqueous heat transfer medium which is liquid from about -73° C. to about 740° C. under atmospheric pressure. This alloy enjoys wide application in heat transfer, power cycles and in other applications where a heat carrying medium which is liquid over a wide temperature range is necessary. The present liquid ternary alloys are possessed of certain physical properties, for example, high heat capacity and thermal conductivity, which properties enhance the value of these alloys for use as heat carrying fluids in many applications.

Broadly, these alloys are comprised of a major amount of cesium, a minor amount of potassium and a small amount of sodium.

More particularly, ternary alloys of this invention, contain by weight from about 2 to about 7% sodium, from about 16 to about 36% potassium and from about 60 to about 80% cesium. Alloys falling within this range of composition are liquid down to at least about -60° C. Between about -60° C. and about -73° C., a small amount of solid phase may appear in the liquid. The eutectic composition has a melting point of about -73° C.

Preferably, the alloys of this invention will contain from about 2.5 to about 4.5% sodium and from about 20 to about 31% potassium and from about 65 to about 77% cesium. These preferred alloys are liquid down to a temperature of at least about -70° C. Below this temperature down to about -73° C., most of the preferred alloy remains liquid but some solid phase is present.

Particularly, preferred alloys are those having the composition of about 2.8% to about 3.2% sodium and from about 20% to about 30% potassium and from about 67% to about 77% cesium. These preferred alloys are completely liquid down to a temperature of at least about -70° C. Our most preferred alloy is that falling within the range of composition of about 70-77% cesium, about 22.5-25.5% potassium and about 2.9-3.1% sodium. This alloy has a composition very close to the eutectic point and is substantially liquid down to a temperature of about -73° C.

The alloys of this invention are prepared by mechanically mixing these metals at a temperature above their melting points in an inert environment. Mixing can be accomplished by agitation, stirring, or other conventional mechanical mixing procedures. Typical inert environments include anhydrous mineral oil or inert gas such as argon, neon, or the like.

FIG. 1 illustrates the phase diagram for the alloys of this invention.

2

FIG. 2 illustrates schematically one preferred embodiment for producing energy according to this invention.

FIG. 3 illustrates schematically an alternative embodiment for producing energy according to this invention.

Referring specifically to FIG. 1, the area bounded by line ABCDA contains the most preferred alloys according to this invention. The alloys having approximately the composition of point A have a melting point between about -72° C. and -73° C. Alloys having the approximate composition of points B, C, and D have melting points of about -70° C. Alloys having a composition falling on line EFGHE have a melting point of approximately -60° C. Alloys having a composition falling within the area bounded by line EFGHE and outside the area bounded by ABCDA, have a melting point between about -60° C. and about -70° C.

Alloys having the composition of this invention are particularly useful in applications wherein it is necessary to store a heat transfer medium under conditions in which it is undesirable or impossible to maintain the storage receptacle in a heated condition. Such conditions occur in many systems, for example, in aircraft and missile applications.

Referring specifically to FIG. 2, which exemplifies one specific application of the alloys of this invention in producing power, an alkali metal alloy of this invention is withdrawn from a mixed metal storage receptacle 10 through a conduit 12 by pump means 14 and is transferred to a fractionator 16 and thence to a boiler 18. In boiler 18, heat from a source 26 is supplied to the alkali metal alloy of this invention. Heat source 26 can be connected to any heat generating source such as steam or molten sodium from an atomic reactor. The alloy of this invention is heated in boiler 18 to the boiling point of cesium (670° C.) whereupon cesium rich vapor is distilled out of boiler 18 upward into fractionator 16. The residue of cesium-lean sodium and potassium left in boiler 18 is conducted by means of a conduit 20 to a mixer 22.

A cesium vapor stream is conducted from fractionator 16 by means of a conduit 24 to a super heater 25. The cesium vapor is supplied with any additional heat as may be required in the super heater 25. If additional heating is not required, super heater 25 can be omitted. The cesium vapor is then conducted by means of a conduit 28 to a power producing means 30 wherein the cesium vapor expends a portion of its energy in the production of power. Any suitable power producing means including, for example, a turbine can be used to produce power. Conventional turbines known to the art are suitable for this purpose. Cesium vapor is expelled through power producing means 30 and is conveyed by means of a conduit 32 to a condenser 34 wherein the cesium vapor is condensed to liquid cesium. Any suitable condensing means can be employed at this stage, it only being necessary that the particular condenser be capable of condensing substantially all of the cesium vapor chosen to cesium liquid.

In mixer 22, the liquid residue of sodium and potassium from conduit 20 is mixed with the liquid cesium from conduit 36 to form the alloy of this invention in the mixer 22. The alloy of this invention is then conveyed by means of conduit 38 to receptacle 10 for storage prior to reuse in the cycle.

In operating the equipment illustrated by FIG. 2, the rate of liquid residue supplied to mixer 22 through conduit 20 and the rate of liquid cesium supplied to mixer 22 through conduit 36 are regulated so that the proper proportions of cesium, sodium and potassium are present in mixer 22 to constitute an alloy of this invention.

The compositions of this invention can be employed

advantageously in a power producing cycle wherein the composition and its individual constituents are the only heat transfer media employed in the entire power generating system.

One advantageous power generating system in which the compositions of this invention can be employed as the sole heat transfer medium is that illustrated in FIG. 3.

According to the process schematically shown in FIG. 3, a fractionator 40 is supplied by a conduit 42 with a liquid binary alkali metal mixture of sodium and potassium. This binary mixture has been heated almost to its boiling point under the pressure of the system by passage through atomic reactor 44. In boiler 46, this binary mixture is contacted with a cesium rich composition supplied through a conduit 48. Fractionator 40 and boiler 46 operate to separate the cesium from the sodium and potassium. The cesium leaves the fractionator 40 as a vapor which is conducted through a conduit 50 to a power producing means 52. In power producing means 52, the excess energy contained within the cesium rich vapor is expended to produce power by a conventional means as, for example, a turbine, a magnetohydrodynamic generator or combinations of these, and the like. Cesium rich vapor is then conducted through a conduit 54 to a condenser 56 wherein the cesium is condensed to its liquid state. The condensed cesium rich liquid is then returned through a conduit 48 and fractionator 40 to boiler 46. Portions or all of this system can be placed under either positive or negative pressure, with respect to atmospheric pressure, as is desired to achieve adequate material and energy balances.

It is necessary to avoid the circulation of any substantial amount of cesium through an atomic reactor because cesium has a relatively high neutron cross section. Sodium and potassium, on the other hand, can be circulated through an atomic reactor without difficulty because they possess relatively low neutron cross sections. If it is desired to use this fluid as a moderator within the reactor, an amount of cesium proportional to the amount of moderation desired can be circulated with the sodium and potassium.

In the specification, claims and specific examples, all parts and percentages are by weight unless otherwise indicated.

In a typical preparation of the eutectic alloy of this invention, molten cesium, potassium and sodium are mixed under an inert atmosphere of argon to produce an alloy having the composition 3.02% sodium, 21.55% potassium and 75.43% cesium, M.P., -72.4° C.

5

10

15

20

25

30

35

40

45

50

50

The following table contains pertinent thermodynamic data comparing the properties of typical alloys of this invention with the properties of sodium, potassium, cesium, mercury and various binary mixtures.

These data show that the alloys of this invention have an extremely low melting point and a very high boiling point. The other physical properties of these alloys render them much more desirable and generally superior to single metals or binary mixtures for use as heat transfer media.

The alkali metals used to prepare the alloys of this invention are commercially available. These commercially available alkali metals are of adequate purity for use in this invention.

The use of cesium in the production of power by means of extracting power from cesium vapor has many advantages. In many applications such as, for example, high temperature nuclear applications, it is necessary to use liquid metals since these are the only materials which are adequately stable under these conditions. Alkali metals are useful in these applications because they have relatively low melting and boiling points and are liquid over wide temperature ranges. For many applications, cesium is particularly desirable because of its very low melting point of 28.5° C. This low melting point means that when cesium is present in its liquid state, excessive heat need not be applied to the cesium to keep it liquid. Also, if the cesium is inadvertently allowed to solidify in the apparatus, it can be rendered molten again without the application of large quantities of heat.

Cesium has many desirable physical properties which make it valuable for use in the production of power. For example, it has a low density and a low heat of vaporization. It is often desirable to operate the power producing process of this invention in such a manner that the initial ternary mixture which is supplied to the boiler is somewhat richer in cesium than those compositions indicated above to be the preferred compositions. When the ternary mixtures of this invention are heated and fractionated to provide cesium vapor for use in producing power, if the initial starting composition is rich in cesium, the vapor which is evolved from the boiler will be substantially pure cesium. Under these conditions, the residue left in the boiler will be a composition which is close to the area defined by line ABCDA in FIG. 1 and will thus enjoy the advantages of a low melting point. In this manner, it is possible to optimize both the advantages of using a substantially pure cesium vapor and developing a residue with a very low melting point.

The equipment utilized in the power producing process

Table I

| Physical Property                            | 100% K    | 100% Na     | 100% Cs   | 100% Hg   | 77% K,<br>23% Na | 23% K,<br>77% Cs | 5% Na,<br>95% Cs | Na-K-Cs Alloy |         |         |
|----------------------------------------------|-----------|-------------|-----------|-----------|------------------|------------------|------------------|---------------|---------|---------|
|                                              | Point A   | Point A     | Point H   |           |                  |                  |                  | Point A       | Point A | Point H |
| Melting Point (° C.)                         | 63.7      | 97.8        | 28.5      | -38.9     | -10              | -48              | -25              | -73.1         | -69.2   | -63.8   |
| Boiling Point (° C.)                         | 760       | 883         | 705       | 357       | 800              | 733              | 746              | 748           | 747     | 763     |
| ΔH Vaporization (cal./g.)                    | 496       | 1,005       | 146       | 69.7      | 613              | 226              | 189              | 247           | 264     | 292     |
| Heat Capacity (cal./g.)                      | 0.189     | 0.31        | 0.060     | 0.0323    | 0.212            | 0.088            | 0.07             | 0.095         | 0.10    | 0.11    |
| (200° C.)                                    |           |             |           | (300° C.) | 2.8              | 17.5             | 6.28             | 4.93          | 6.8     | 7.3     |
| ΔH Fusion (cal./g.)                          | 14.6      | 27.1        | 3.766     |           |                  |                  |                  |               |         | 8.1     |
| Density (g./cc.)                             | 0.783     | 0.891       | 1.84      | 13.1      | 0.75             | 1.27             | 1.80             | 1.58          | 1.53    | 1.50    |
| Viscosity (centipoises)                      | 0.26      | 0.381       | 0.3430    | (28° C.)  | 1.01             | 0.30             | 0.352            | 0.310         | 0.303   | 0.311   |
| (250° C.)                                    | (250° C.) | (210.9° C.) | (200° C.) | (200° C.) |                  |                  |                  |               |         |         |
| Thermal Conductivity (cal./sec.-cm.<br>° C.) | 0.10      | 0.1974      | 0.044     | 0.0303    | 0.133            | 0.072            | 0.080            | 0.085         | 0.087   | 0.098   |
| (300° C.)                                    | (200° C.) | (at M.P.)   | (220° C.) |           |                  |                  |                  |               |         |         |
| Wt. Percent                                  |           |             |           |           |                  |                  |                  |               |         |         |
| Point                                        | A         | B           | H         |           |                  |                  |                  | A             | B       | H       |
| Na                                           | 3.02      | 2.93        | 6.13      |           |                  |                  |                  | 10.5          | 9.5     | 18.3    |
| K                                            | 21.55     | 26.67       | 26.67     |           |                  |                  |                  | 44.1          | 50.5    | 47.0    |
| Cs                                           | 75.43     | 70.40       | 67.20     |           |                  |                  |                  | 45.4          | 39.6    | 34.7    |

of this invention can be relatively light-weight because excessively high pressures are not involved. Furthermore, since cesium has a comparatively low boiling point, the temperatures encountered in this process are not such that excessive precautions are necessary to prevent the cesium vapor from attacking the equipment. When a turbine is used as the power producing means, it is possible to use a turbine having only two stages and a small rotor diameter to absorb the enthalpy drop with cesium. This type of turbine is compact and lightweight which are important advantages in missile, aircraft and spacecraft applications.

The ternary compositions of this invention constitute highly desirable heat transfer media because of their relatively low melting and high boiling points coupled with good heat capacity and thermal-conductivity. The extremely low melting points of these alloys render them particularly desirable for use in applications in which it is impossible or impractical to maintain a heat transfer medium in a heated condition to prevent its solidification. The ternary mixtures of this invention are liquids having substantially constant physical and chemical properties over a temperature range of almost 800° C.

As will be understood by those skilled in the art, what has been described is the preferred embodiment of the invention; however, many modifications, changes and substitutions can be made therein without departing from the scope and the spirit of the following claims:

What is claimed is:

1. The method comprising heating a ternary mixture of sodium, potassium and cesium to provide a stream of cesium rich vapor and a liquid residue, extracting energy from said vapor, condensing said cooled vapor to liquid cesium, admixing said liquid cesium with said liquid residue, the resulting mixture of said liquid cesium with said liquid residue having the composition of said ternary mixture.

2. The method comprising vaporizing a portion of a first mixture of sodium, potassium and cesium to provide

5 a stream of cesium rich vapor and a liquid residue, extracting energy from said vapor, condensing said vapor to a cesium rich liquid, admixing said cesium rich liquid with said liquid residue, the resulting mixture of said cesium rich liquid with said liquid residue having substantially the composition of said first mixture, said first mixture containing from about 2 to about 7% sodium, from about 16 to about 36% potassium and from about 60 to about 80% cesium.

10 3. Process for producing power which comprises: supplying a liquid mixture of sodium, potassium and cesium metals to a vaporizing zone, vaporizing a portion of said mixture in said zone to produce cesium-rich vapors and a cesium-lean liquid residue, employing said vapors to produce power, and thereafter condensing said vapors and combining the condensate with said residue to form said mixture.

15 4. Process for producing power which comprises: fractionating a ternary mixture of cesium, potassium and sodium metals to produce a cesium-rich vapor and a liquid binary mixture of potassium and sodium, employing said vapor to produce power, contacting said liquid with a source of heat to produce a heated liquid binary mixture, and condensing said vapor and combining the condensate with said heated binary mixture to form said ternary mixture.

#### References Cited by the Examiner

#### UNITED STATES PATENTS

|    |           |       |               |       |          |
|----|-----------|-------|---------------|-------|----------|
| 30 | 2,102,424 | 12/37 | Larrecq       | ----- | 60—36 X  |
|    | 2,806,785 | 7/56  | Doptoglone    | ----- | 75—134 X |
|    | 2,911,297 | 11/59 | Florenz       | ----- | 75—135   |
|    | 2,919,189 | 12/59 | Nossen et al. | ----- | 75—135   |
| 35 | 3,040,528 | 6/62  | Tabor et al.  | ----- | 60—36    |
|    | 3,095,698 | 7/63  | Stern         | ----- | 60—36    |

JULIUS E. WEST, *Primary Examiner.*

DAVID L. RECK, EDGAR W. GEOGHEGAN,  
*Examiners.*